

3,834,871

## DURABLE PRESS TEXTILE MATERIALS BY ANHYDROUS SOLVENT FINISHING PROCESS

Jimmy M. Thompson, Salisbury, N.C., assignor to Proctor Chemical Company, Inc., Salisbury, N.C.

No Drawing. Filed Jan. 5, 1972, Ser. No. 215,626  
Int. Cl. D06m 13/12, 13/34

U.S. CL. 8—187

11 Claims

### ABSTRACT OF THE DISCLOSURE

Anhydrous solvent finishing processes to impart durable press properties to cellulosic textile materials, e.g., flat goods or finished garments made of 100% cotton fiber or cotton/synthetic fiber blends, involve impregnating textile material with an anhydrous mixture of methyloated carbamate, organic solvent and organic aminoplast cross-linking catalyst, removing solvent, exposing the solvent-depleted textile material to water vapor to give a moisture regain of 8 to 15% and then heat curing at about 120° to 200° C. The anhydrous organic solvent mixture may include a soluble fire-retardant so that the resulting fabric acquires both durable press and fire retardancy properties.

### BACKGROUND OF THE INVENTION

#### Field of the Invention

The invention relates to the finishing of fabrics and other textile materials made of cellulosic fibers to impart durable press qualities thereto. More particularly, it concerns anhydrous solvent finishing methods for cellulosic textile materials capable of creating high durable press ratings for the textile material and, in some embodiments, simultaneously also creating good fire-retardancy.

#### Description of the Prior Art

Textile articles that can be laundered or cleansed and still maintain an unwrinkled, finished appearance are much in demand. At the present time, a major portion of garments, sheets, pillow cases and other white goods and related textile articles used by people in daily activities and in their households are of this type. A variety of terms have been used to refer to textile materials which can be laundered or cleansed without requiring a substantial amount of ironing or pressing in order for the textile article to have a sufficiently good appearance to be put right back into use after the laundering or cleansing. The term "wash-wear" has been used extensively to describe such textile materials. They have also been referred to as "durable press" articles, particularly in describing finished garments. Other terms have also been employed, some being more extensively used in scientific fields while others are more popular with laymen. The present invention relates to that class of textile materials which resist creasing or other alteration in appearance when subjected to repeated launderings or cleansings sufficiently that they may be returned to their intended use or service without requiring ironing or pressing, except possibly so-called "touch-up" ironing to provide a completely renewed appearance. This type of textile material which will, for the sake of consistency and brevity, be referred to hereinafter as a durable press textile material.

Durable press properties in textile articles can be obtained in a variety of ways. Some fibers and fabrics exhibit much less tendency towards creasing or developing an unacceptable appearance than do other fibers or fabrics. For example, knit goods made of certain synthetic fibers require less attention to restore satisfactory appearance than do woven fabrics made of natural fibers. A principal method of imparting durable press properties to textile articles

is by treating a fabric or a finished garment with some form of crease-proofing agent.

An enormous amount of research and development work has been devoted to the improvement of durable press textile articles while mitigating adverse effects such as loss of tensile strength or abrasion resistance, lowering the cost of production and manufacture or the like. In large measure, this has involved investigation of numerous types of crease-proofing agents, methods of treating textiles with them, catalyst systems used in such methods and the like. Ureaformaldehyde resins, melamine-formaldehyde resins and a multitude of other nitrogen containing resins or their precursors, broadly referred to as aminoplasts, constitute one of the major types of materials used as crease-proofing agents for cellulosic textile materials. They are applied almost exclusively to fibers and fabrics from aqueous systems, i.e., solutions or dispersions of the agents in water or liquids containing a substantial amount of water. In addition to the durability problems, i.e., reduction in abrasion resistance and tensile strength, many of the agents of this class also create a "chlorine-retention" problem, i.e., accumulation of chlorine in the fabric following the application of chlorine containing bleaches due to the presence in the fabric of a crease-proofing agent. This latter deficiency has in large measure been eliminated by the use of monocyclic urea derivatives as agents for providing the desired durable press properties (see U.S. 2,373,135).

One class of chemical compounds which have been found to provide relatively high durable press values with relatively low detrimental side effects are methyloated carbamates (see U.S. 3,144,299). These have been applied to fibers of fabrics from aqueous systems and special catalysts have been developed for use in such operations (see U.S. 3,369,585). Modifications of such operations have included use of special combinations of carbamate treating agents (see U.S. 3,548,427). The utilization of carbamates in this manner has become so extensive that improved procedures for producing and manufacturing methyloated carbamates have been developed (see U.S. 3,391,181). The present invention concerns improved procedures for imparting durable press properties to cellulosic textile materials using methyloated carbamates.

Non-aqueous systems have been used to a limited extent for the treatment of textile materials with crease-proofing agents. For example, solutions of treating agents in organic solvents may be employed for impregnation of textile materials where the agent is either completely insoluble in water or will decompose if brought into contact with water. In such cases, the organic solvent solution can be employed to place the treating agent in or upon the fabric after which an aqueous-treating system may be applied (see U.S. 3,508,860). In other cases, non-aqueous solutions of treating agents in organic solvents that have a swelling action on fibers comparable to water have been used to apply treating agents to fibers and fabrics (see U.S. 2,161,805).

The use of aminoplasts as crease-proofing agents depends, at least in part, in a cross-linking reaction between hydroxyl groups in the cellulosic fibers of the textile material and methyloled or equivalent groups in the aminoplasts. Many aminoplasts can also undergo condensation polymerization creating resinous materials within the fiber or fabric which to some extent contribute to durable press properties imparted to the textile material. However, a large number of the effective nitrogen containing crease-proofing agents, including the methyloated carbamates, do not polymerize to form resinous materials and their crease-proofing characteristics are due to a cross-linking action upon the cellulosic fibers of the textile materials. In contrast, there are operations for

3  
producing durable press fabrics in which fabrics are treated with resin forming substances that are not reactive with the cellulosic fibers so that crease-proofing effects are due entirely to the formation in the fabric of resinous materials. Unsaturated organic compounds, e.g., acrylic acid esters, capable of undergoing free-radical type polymerization have been used for this purpose. Such polymerized unsaturated compounds are usually water-insoluble and solutions of such compounds in organic solvents are frequently used to apply an unsaturated compound to a textile material so that it may be polymerized in situ upon the textile material (see U.S. 2,071,419).

### OBJECTS

A principal object of this invention is the provision of new improvements in the production of durable press textile materials. Further objects include the provision of:

(1) New methods for treating cellulosic textile materials with non-aqueous crease-proofing compositions to impart durable press properties.

(2) New finishing processes for cellulosic textile materials to impart durable press properties which may be applied to 100% cotton fiber fabrics.

(3) New durable press treatments for cellulosic textile materials that can simultaneously impart fire-retardancy to the textile material.

(4) New forms of cellulosic textile materials that exhibit high durable press ratings along with satisfactory tensile strength and abrasion resistance.

(5) New anhydrous, organic solvent compositions for use in the finishing of cellulosic textile materials to impart durable press properties.

Other objects and further scope of applicability of the present invention will become apparent from the detailed description given hereinafter; it should be understood, however, that the detailed description, while indicating preferred embodiments of the invention, is given by way of illustration only, since various changes and modifications within the spirit and scope of the invention will become apparent to those skilled in the art from this detailed description. It should also be understood the foregoing abstract of the disclosure is for the purpose of providing a non-legal brief statement to serve as a searching-scanning tool for scientists, engineers and researchers and is not intended to limit the scope of the invention as disclosed herein nor is it intended it should be used in interpreting or in any way limiting the scope or fair meaning of the appended claims.

### SUMMARY OF THE INVENTION

These objects are accomplished in accordance with the present invention by treatment of cellulosic textile materials with methylolated carbamates applied as solutions in anhydrous, organic solvents in combination with organic compounds which are soluble in the organic solvent and function as aminoplast cross-linking catalysts. The success of the invention is due, at least in part, to the discovery that when methylolated carbamates are applied to cellulosic textile materials from anhydrous solvent media, there can be substantial improvement in the overall properties of the treated material as contrasted to results obtained using aqueous systems. Further, the curing of the fabric to produce reaction between the methylolated carbamate and cellulosic fibers of the textile material to generate the durable press effect can be accomplished in very short time so that the new operations can be used in mills for normally fast continuous processing.

Stated briefly, processes for the production of durable press cellulosic textile materials in accordance with the invention involve the following steps:

(A) Providing a substantially anhydrous mixture comprising the following:

(a) methylolated carbamate,

4  
(b) organic solvent having a boiling point between about 50° and 200° C.,  
(c) organic aminoplast cross-linking catalyst soluble in said organic solvent,

5  
10 (B) Impregnating cellulosic textile material with said anhydrous mixture to provide in the textile material between about 1 and 10% of said methylolated carbamate based upon the dry weight of said textile material,

(C) Removing organic solvent from the impregnated textile material resulting from step B,

(D) Exposing the solvent-depleted textile material of step C to water vapor to create therein a moisture regain of between about 8 to 15% in the cellulosic fibers of the fabric.

(E) Heating the textile material resulting from step D at a temperature between about 120° and 200° C. for a time between about 1 and 30 minutes sufficient to produce an increased durable press rating in said textile material.

20 The anhydrous solvent finishing processes of the invention appear to be usable with any methylolated carbamates which have been found to be effective in creating durable press properties in cellulosic textile materials. However, particularly useful results have been obtained in accordance with the invention using methylolated carbamates of the formula:



30 wherein

R<sub>1</sub> is X or Y

X is —R<sub>2</sub> or —R<sub>3</sub>—O—R<sub>2</sub>

35 Y is



40 R<sub>2</sub> is 1 to 4 carbon atom alkyl,

R<sub>3</sub> is 1 to 20 carbon atom alkyne,

R<sub>4</sub> is —H or —R<sub>2</sub>, and

45 R<sub>x</sub> is —CH<sub>2</sub>OH when R<sub>1</sub> is X or —CH<sub>2</sub>OH or R<sub>4</sub> when R<sub>1</sub> is Y.

A preferred class of the methylolated carbamates are those having the following formula:



50 wherein:

Z is —H, —R<sub>2</sub> or —CH<sub>2</sub>OH,

R is —R<sub>2</sub> or —R<sub>5</sub>—O—R<sub>2</sub>,

55 R<sub>2</sub> is 1 to 4 carbon atom alkyl, and

R<sub>5</sub> is 1 to 4 carbon atom alkyne.

60 As the organic solvent of the anhydrous systems used in accordance with the invention, halogenated hydrocarbons are advantageous not only because they are highly effective in the operations but also from a safety viewpoint if non-flammable halogenated hydrocarbons are used. However, the new methods are effective with the use of other water-immiscible organic solvents including hydrocarbons, esters and ethers. The anhydrous solvent may contain up to about 10% of an aliphatic alcohol or an alkoxyalkane to improve the solubility of the methylolated carbamate used in the anhydrous system as the durable press producing agent.

65 As to the catalyst used to promote cross-linking between the methylolated carbamate and the cellulosic fibers, a variety of organic solvent soluble compounds having cross-linking catalytic effect on aminoplasts are known and can be used. Advantageously, from among these a catalyst will be selected which does not adversely affect

fabric strength, color or other desired qualities. By way of example, p-toluene sulfonyl chloride has been found particularly useful. Preferred catalysts are those selected from the group consisting of haloaryllacetones, halimides and aryl sulfonyl halides.

Success of the invention is, in part, further due to the discovery that durable fire-retardant properties can be produced in cellulosic textile materials simultaneously with durable press properties using the same anhydrous solvent systems as outlined above relative to the durable press agent. Halogenated hydrocarbyl phosphates constitute a preferred type of fire-retardant agent for use in these new textile treatments. However, a variety of other fire-retardants may be employed as disclosed hereinafter and also in copending application S.N. 292,145, filed Sept. 25, 1972, the disclosure of which is incorporated herein by reference.

#### DESCRIPTION OF PREFERRED EMBODIMENTS

The following details of operations in accordance with the invention and reported data illustrate the further principles of practice of the invention to those skilled in the art. In these examples and through the remaining specification and claims, all parts and percentages are by weight unless otherwise specified.

##### Example I

A clear solution was prepared by mixing together, in the parts specified, the following ingredients and stirring them until a stable solution was obtained:

|                                         | Parts |
|-----------------------------------------|-------|
| N,N-dimethylol-2-methoxyethyl carbamate | 125   |
| p-Toluene sulfonyl chloride             | 10    |
| Isopropanol                             | 10    |
| Methoxyethanol                          | 10    |
| 1,1,1-trichloroethane                   | 845   |

A section of 100% cotton broadcloth fabric was immersed in the resulting solution until it was thoroughly impregnated. It was then pad-squeezed to a wet pick-up of 80%, after which it was dried at room temperature (20-25° C.) for 10 minutes resulting in substantially complete evaporation of the trichloroethane. Next the fabric section was wet steamed to a moisture regain of 8-15% and then immediately subjected to a hot air cure cycle of 1.5 minutes at 170° C. After being removed from the hot air oven, the fabric section was conditioned to ambient temperature and humidity and then subjected to several standard fabric testing procedures. This produced the following data:

Crease Recovery (AATCC No. 66—Recovery Angle Method) (warp and filling)=280°+  
Durable Press Rating (AATCC No. 124—Durable Press Replica) after 50 home launderings=3.8-4.2

##### Example II

As an Example I, a clear solution was made of the following ingredients:

|                                | Parts |
|--------------------------------|-------|
| N,N-dimethylol ethyl carbamate | 125   |
| Benzene sulfonyl chloride      | 10    |
| n-Propanol                     | 10    |
| Methoxyethanol                 | 10    |
| Perchloroethylene              | 845   |

A section of 100% cotton broadcloth was impregnated with the solution and then pad-squeezed to a wet pick-up of 80%. The fabric was then dried in forced air oven at 100° C., immediately steamed to a moisture regain of 8-15% and then given a hot air cure for 3 minutes at 160-165° C. The ambient conditioned fabric when tested produced the following data:

Crease Recovery=270°+  
Durable Press Rating=3.8-4.0 (50 launderings)

#### Example III

As in Example I, a clear solution was made of the following ingredients:

|                                             | Parts |
|---------------------------------------------|-------|
| N,N-dimethylol tetrahydrofurfural carbamate | 125   |
| p-Toluene sulfonyl chloride                 | 10    |
| n-Propanol                                  | 10    |
| Trichloroethylene                           | 855   |

A 50/50 polyester/cotton broadcloth was impregnated by pressure spray application to produce a wet pick-up of 65%. The fabric was then passed over low pressure (30-40 p.s.i.g.) steam cans to produce solvent evaporation and dry the fabric. This was then followed by light steaming to produce a moisture regain of 8-15% in the cellulose fibers of the fabric. Finally, the fabric was cured for 1 minute at 160-165° C. The ambient conditioned fabric when tested produced the following data:

Crease Recovery=280°+  
Durable Press Rating=4.0-4.2 (50 launderings)

#### Example IV

As in Example I, a clear solution was made of the following ingredients:

|                                         | Parts |
|-----------------------------------------|-------|
| N,N-dimethylol-2-methoxyethyl carbamate | 125   |
| p-Toluene sulfonyl chloride             | 10    |
| Tris (2,3-dibromopropyl) phosphate      | 250   |
| Methoxy methyl melamine                 | 50    |
| 1,1,1-trichloroethane                   | 565   |

A 100% cotton broadcloth was impregnated with the solution and the pad-squeezed to a wet pick-up of 80%. The fabric was air dried at room temperature for 10 minutes and then lightly steamed to produce a moisture regain of 10-15%. Finally, the fabric was cured for 1 minute at 160-165° C. The ambient conditioned fabric when tested produced the following data:

Crease Recovery=278°  
Durable Press Rating=4.0 (one laundering)  
Durable Press Rating=3.8-4.0 (50 launderings)  
Vertical Char (AATCC No. 34-1969)=4.5" (one laundering) no flame or after glow  
Vertical Char=7-8" (50 launderings) no flame or after glow

#### Example V

As in Example I, a clear solution was made of the following ingredients:

|                                         | Parts |
|-----------------------------------------|-------|
| N,N-dimethylol-2-methoxyethyl carbamate | 150   |
| p-Toluene sulfonyl chloride             | 10    |
| Tris (2,3-dibromopropyl) phosphate      | 200   |
| Methoxy methyl melamine                 | 50    |
| 1,1,1-trichloroethane                   | 615   |

A 100% viscose rayon prepared fabric impregnated with the solution to a wet pick-up of 70%. The fabric was dried by solvent evaporation for 10 minutes at room temperature and then lightly steamed to a moisture regain of 8-15%. Finally the fabric was hot air cured for 1 minute at 160-165° C. The ambient conditioned fabric when tested produced the following data:

Crease Recovery=265°  
Durable Press Rating=3.8 (one laundering)  
Durable Press Rating=3.5 (50 launderings)  
Vertical Char=4.5" (one laundering) no flame or after glow  
Vertical Char=7.0" (50 launderings) no flame or after glow

7  
Example VI

As in Example I, a clear solution was made of the following ingredients:

|                                         | Parts |
|-----------------------------------------|-------|
| N,N-dimethylol-2-methoxyethyl carbamate | 125   |
| p-Toluene sulfonyl chloride             | 10    |
| Tris (2,3-dibromopropyl) phosphate      | 350   |
| Methoxy methyl melamine                 | 50    |
| 1,1,1-trichloroethane                   | 465   |

A 50/50 polyester/cotton prepared sheeting fabric (percale) was impregnated with the solution to a wet pick-up of 60% and then allowed to dry at room temperature by solvent evaporation. The dry fabric was steamed to a moisture regain of 8-15% based upon the weight of the cellulosic component of the fabric. Finally, the fabric was hot air oven cured for 1 minute at 160-165° C. The ambient conditioned fabric when tested produced the following data:

Crease Recovery=285°  
Durable Press Rating=4.5 (one laundering)  
Durable Press Rating=4.5 (30 launderings)  
Vertical Char=5.5" (one laundering)  
Vertical Char=8-9" (30 launderings)

## DISCUSSION OF DETAILS

The new anhydrous solution methods for treatment of cellulosic textile articles to obtain durable press effects are contemplated for use with all methylolated carbamates known to be useful as crease-proofing agents for cellulosic fabrics. Such reagents are discussed in numerous publications and patents, e.g., see U.S. Pats. 3,219,686; 3,369,858; 3,391,181; 3,548,427 and 3,553,254 the disclosures of which are incorporated herein by reference. N,N-dimethylol alkoxy alkyl carbamates as hereinbefore defined are particularly useful, e.g., N,N-dimethylol-2-methoxyethyl carbamate. Specific examples of other carbamates preferred for use in the new methods include the N,N-dimethylol derivatives of the following carbamates:

|                              |                          |
|------------------------------|--------------------------|
| ethyl carbamate              | octadecyl carbamate      |
| tetrahydrofurfural carbamate | cyclohexyl carbamate     |
| allyl carbamate              | n-propyl carbamate       |
| 2-ethyl hexyl carbamate      | isopropyl carbamate      |
| 2-chloroethyl carbamate      | hydroxyethyl carbamate   |
| 3-bromopropyl carbamate      | phenyl carbamate         |
| 3-ethoxypropyl carbamate     | p-chlorophenyl carbamate |
| 6-methoxyhexyl carbamate     | p-tolyl carbamate        |

Additional examples of specific carbamates useful in the new operations include:

|                                                  |
|--------------------------------------------------|
| N,N'-dimethylol ethylene bis (ethyl carbamate)   |
| N,N'-dimethylol butane-1,3-diol dicarbamate      |
| N,N'-dimethylol diethylene glycol dicarbamate    |
| polymethylol pentaerythritol tetracarbamate      |
| N,N',N'-trimethylol glycerol tricarbamate        |
| polymethylol sorbital hexakis (methyl carbamate) |
| N,N'-dimethylol-2,4-pentane-1,5-diol dicarbamate |

The halogenated hydrocarbons having a boiling point between about 20-200° C. and especially between about 50-150° C., are a preferred class of anhydrous organic solvents for use in the new DP fabric treatments, e.g., 1,1,1-trichloroethane, butyl bromide, perchloroethylene, trichloroethylene, ethylene chloride, ethylene bromide, 1,1,2-trichloro-1,2,2-trifluoroethane, 1,1,1-trichloro-2,2,2-trifluoroethane, methyl chloride and 1,1-dichloroethane. Other anhydrous organic solvents of similar boiling range may, however, be used including hexane, pentene-1, methyl ethyl ketone, isopropyl acetate, ethyl acetate, isopropyl ether, ethyl formate, neohexane, dioxolane, cyclohexane, cyclopentane, benzene, acetone and the

like. Mixtures of two or more anhydrous organic solvents may also be used with advantage, particularly where it is desired to control evaporation or drying rate of the fabric treatment solution from the impregnated textile material.

5 A wide selection of aminoplast catalysts soluble in anhydrous organic solvents are available for use in the new DP treatments. Advantageously, one selects such a catalyst that will not stain or discolor the fabric, cause excessive tendering or present safety or pollution problems. 10 Aromatic sulfonyl halides have been found to be particularly useful, e.g., p-toluene sulfonyl chloride, benzene sulfonyl chloride, 2-chloro-4-ethylphenyl sulfonyl chloride, benzene sulfonyl bromide and the like. The catalyst that is used should be soluble at least to the extent of 1% in the organic solvent hereinbefore described. Advantageously, compounds used as the catalyst are acidic or react with water to form an acidic product. Additional preferred classes of compounds to use as catalysts include halogenated aromatic lactones, e.g., chlorophthalide, bromophthalide, iodophthalide, etc. and haloimides, e.g., N-chlorosuccimide, N-bromo- $\alpha$ , $\beta$ -dibromo succimide, N-chloro teraconimide, N-chlorophthalimide and the like. The amount of catalyst used will depend, in part, upon the 15 particular carbamate reagent used, the temperature for curing and similar factors. Generally, the fabric treating solution will comprise 0.1 to 10% of the catalyst and especially 0.1 to 5%.

Two major components of the anhydrous textile treating 30 solution of the invention are methylolated carbamate and organic solvent. Such solutions may contain 1 to 50% methylolated carbamate or carbamate mixtures, and particularly 5 to 20%, catalyst in amount as aforesaid and the remainder organic solvent, e.g., 40 to 98% solvent. 35 Advantageous solutions comprise 5 to 20% carbamate component, 0.1 to 5% catalyst and the remainder organic solvent of which at least 90% is halogenated hydrocarbon or mixture, particularly halogenated hydrocarbons of 2 to 3 carbon atoms.

The organic solvent component of the treating solution may contain up to about 10%, e.g., 1-5%, of organic hydroxy compound to improve solubility of the carbamate component. Alkanols of 1-6 carbon atoms, e.g., ethanol, isopropanol, n-butanol, tert-butanol, methanol, hexanol, etc. or alkoxyalkanols of 3-8 carbon atoms, e.g., methoxyethanol, ethoxyethanol, butoxybutanol, methoxyhexanol, etc. are useful for this purpose. Mixtures of such organic hydroxy compounds may advantageously be used within the amounts indicated.

50 As illustrated by Examples IV to VI, a third major component of the new anhydrous treating solution may be a fire-retardant. Such component when used may comprise up to 60% of the treating solution and may, in part, serve as a solvent vehicle for the carbamate component.

55 Any anhydrous organic compounds known to be useful as fire-retardants are contemplated for use as components of the treating solutions, e.g., see "Chem. and Eng. News," Oct. 18, 1971, p. 16-19. Organic chlorine compounds, bromine compounds, nitrogen compounds and phosphorus compounds having flame-proofing qualities are usable if they are non-reactive with the carbamate component. Advantageously, the treating solutions of the invention, when fire-retardancy as well as DP effects are desired, will contain 5 to 40% of the flame-proofing agent. Preferred 60 solutions of this type will comprise 5 to 20% carbamate component, 10 to 30% fire-retardant, 0.1 to 5% catalyst, 20 to 80% anhydrous organic solvent and up to 20% of an auxiliary reagent.

Auxiliary reagents of various types may be included in the 65 treating solutions, advantageously in amounts between 0.1 to 20% and particularly between 0.5-15%, especially 1-10%. Such auxiliary reagents include dyes; thermosetting resins, e.g., methyl and butyl ethers of dimethylol derivatives of triazines; ethylene urea, melamine, propylene urea, etc.; mildew-proofing agent; sanitizing agents;

softening agents, plasticizers; hand-builders and the like. The DP treatments of the invention are usable with all varieties of cellulosic textile materials. The term "cellulosic textile material" as used herein is intended to mean any woven, knit or non-woven fabric as well as garments, bed-clothes, furniture coverings or any other textile material made in whole or in part of cellulosic fibers. Cellulosic fibers include cotton, linen, viscose rayon, high modulus rayon (polynosic). These may be blended in yarns with synthetic fibers, e.g., nylon, polyester, polyolefin and other fibers or filaments or the textile materials may comprise mixed weaves or knits of cellulosic yarns or filaments and synthetic yarns or filaments. A particular advantage of the invention is the ability of the new operations to impart DP effects to 100% cotton textile materials without undue loss of tensile strength and abrasion resistance.

The anhydrous treating solutions of the invention may be applied in a variety of ways. Dipping and padding, well known in the art, can be used. Additional methods include spraying, roller coating, float coating and the like. However, if enclosed equipment is not used, loss of solvent to the atmosphere can be costly and/or present ecological problems. Equipment is commercially available to perform the application of organic solvent treating solutions without loss of solvent to textile material, e.g., see "Textile Industries," October 1966, pp. 288-9, 291, 295, 299, 339 and 397.

The amount of solution applied will depend upon the type of fabric, e.g., whether woven or knit and its weight, the degree of DP effect desired, the concentration of carbamate in the solution and similar factors. Under preferred conditions, the amount of solution relative to textile material will be selected to provide in the textile material between about 1-20%, especially 1-10%, of carbamate component based upon the dry weight of the cellulosic textile material. Typically, this will involve a wet pick-up of treating solution between about 50-150% based upon the dry weight of the textile material.

Following the application of the anhydrous treating solution, the volatile components of the solution are removed, e.g., by evaporation. Passage of the textile material through drying ovens, through infra-red ovens or in any other suitable manner may be used. The evaporated organic solvent is removed and recovered with available solvent handling systems. As a less desirable alternative, the impregnated textile material may be permitted simply to air dry at ambient conditions.

The removal of the organic solvent from the textile material leaves a moisture and solvent depleted fabric. At this point in the new operations, the solvent depleted fabric is exposing to water vapor to create therein a moisture regain in the cellulosic portion of the fabric of between about 8 and 15%. For 100% cotton, this will mean a total moisture regain of 8-15% while a 50% cotton/50% polyester fabric would involve a total moisture regain of 4-7.5%. Advantageously, this is accomplished by steaming of the textile material. Exposure to high humidity at room temperature or other moisture regain techniques can, however, be used. As an alternative, the moisture regain step may be applied before the solution application or before the solvent evaporation steps. However, more pronounced DP effects are obtained when the moisture regain step is applied after the solvent evaporation. This also improves solvent recovery operations. The moisture regain step appears to be necessary to the success of the new methods, at least in part, to produce ionization of the acidic catalyst to produce the curing of the impregnated textile material.

The textile material ultimately is subjected to a heat curing step to produce cross-linking of the cellulosic fiber components with the methylolated carbamate. This heat curing may proceed immediately after the combination of solution application and moisture regain. Alternatively, a delay cure procedure may be used. In any event, heat

curing equivalent to 1-30 minutes at 120° to 200° C. is used to sufficiently produce an increased durable press rating in the textile material as compared to untreated textile material.

#### CONCLUSION

New anhydrous organic solvent procedures have been described for treatment of cellulosic textile materials to obtain durable press effects. These new techniques enhance, rather than diminish the over-all properties of the fabric. Moreover, the procedures may be operated to attain durable fire-retardancy as well as DP effects. Further, the curing of the textile material can be effected in a very short time so that the new operations are usable in textile mills requiring fast, continuous processing of fabrics.

The embodiments of the invention in which are exclusive property or right is claimed are defined as follows:

1. A process for the production of durable press cellulosic textile materials which comprises:

(A) providing a substantially anhydrous mixture comprising the following ingredients in the percentages by weight indicated:

- (a) 5 to 20% methylolated carbamate
- (b) 0.1 to 5% organic aminoplast cross-linking catalyst selected from the group consisting of haloaryllactones, haloimides and aryl sulfonyl halides,
- (c) remainder being organic solvent having a boiling point between about 50° and 200° C. comprising at least 90% of halogenated hydrocarbon containing 2 to 6 carbon atoms,

(B) impregnating cellulosic textile material with said anhydrous mixture to provide in the textile material between about 1 and 10% of said methylolated carbamate based upon the dry weight of said textile material,

(C) drying said textile material resulting from step B by evaporation of said organic solvent,

(D) exposing the dried textile material from step C to water vapor to create therein a moisture regain of between about 8 and 15%,

(E) heating the textile material at a temperature between about 120 and 200° C. for a time between about 1 and 30 minutes sufficient to produce an increased durable press rating in said textile material.

2. The process of claim 1 wherein said methylolated carbamate has the formula:



wherein:

55 R<sub>1</sub> is X or Y,  
X is —R<sub>2</sub> or —R<sub>3</sub>—O—R<sub>2</sub>  
Y is



60 R<sub>2</sub> is 1 to 4 carbon atom alkyl,  
R<sub>3</sub> is 1 to 20 carbon atom alkylene,  
R<sub>4</sub> is —H or —R<sub>2</sub>, and  
R<sub>x</sub> is —CH<sub>2</sub>OH when R<sub>1</sub> is X or —CH<sub>2</sub>OH or R<sub>4</sub> when R<sub>1</sub> is Y.

65 3. The process of claim 1 wherein said methylolated carbamate has the formula:





UNITED STATES PATENT OFFICE  
CERTIFICATE OF CORRECTION

Patent No. 3,834,871

Dated September 10, 1974

Inventor(s) Jimmy M. Thompson

It is certified that error appears in the above-identified patent and that said Letters Patent are hereby corrected as shown below:

Column 1, line 47, "or", first occurrence, should be -- of --.

Column 2, line 59, "in", second occurrence, should be -- to --.

Column 3, line 36, the period after "however" should be a comma;

Column 5, line 4, "haloaryllacetones" should be  
--haloaryllactones--;

Column 7, line 44, "carbamatecyclohexyl" should be  
-- cyclohexyl carbamate --.

Column 9, line 23, "atmoshpere" should be --atmosphere--;

Column 10, between lines 15 and 16, insert the heading  
--Claims--;

Column 10, line 16, "are" should be --an--.

Signed and sealed this 24th day of December 1974.

(SEAL)

Attest:

McCOY M. GIBSON JR.  
Attesting Officer

C. MARSHALL DANN  
Commissioner of Patents